

Jan. 17, 1933.

L. G. GABRIEL

1,894,617

BITUMINOUS EMULSION

Filed June 5, 1928

*Fig. 1.*



*Fig. 2*



INVENTOR

*Leonard Gowan Gabriel*  
*By*  
*Byrnes, Stobbs & Carmelco*  
*His Atty.*

## UNITED STATES PATENT OFFICE

LEONARD GOWEN GABRIEL, OF LONDON, ENGLAND, ASSIGNOR, BY MESNE ASSIGNMENTS, TO COLAS ROADS INC., OF BOSTON, MASSACHUSETTS, A CORPORATION OF MASSACHUSETTS

## BITUMINOUS EMULSION

Application filed June 5, 1928, Serial No. 283,088, and in Great Britain May 22, 1928.

This invention relates to the manufacture of aqueous emulsions of bitumen. Such emulsions are now used to a large extent in the laying and repair of roads and in the preparation of bitumen-coated mineral aggregates for use in road-making.

To be satisfactory for the above and other allied uses, the emulsion must be sufficiently stable in bulk to resist disruption during transportation and storage and on the other hand, when applied to a mineral aggregate, road surface or other foundation, the emulsion must be capable of breaking down rapidly and yielding (by the separation of the aqueous phase) a permanent water-resistant coating of bitumen. This combination of stability and instability shall be referred to herein as the "balance" of stability.

The balance of stability in an emulsion is governed by the size of the dispersed bitumen particles. Generally speaking a reduction in the size of the particles means increased bulk stability but is accompanied by a corresponding reduction in the instability factor, that is to say a reduction in the facility and speed with which the emulsion breaks when applied to a porous surface. Conversely an increase in the size of the particles diminishes the bulk stability but gives an emulsion with a quicker "break" on application. In emulsions which possess the required balance of stability and are now in general use the size of the greater proportion of the bitumen particles is of the order of  $3\mu$ .

One feature of this invention resides in the manufacture of a bituminous emulsion which has the required balance of stability and in which a substantial proportion of the dispersed particles are of a size (e. g.  $10\mu$ ) considerably greater than obtaining in the aforesaid emulsions now generally used.

In British Specification No. 238,967 there is described a process of making a bituminous emulsion which comprises the treatment in a colloid mill of a mixture of molten or liquid bituminous material, a proportion in the region of  $1\frac{1}{2}\%-2\%$  (reckoned by weight on the bitumen) of an emulsifying agent comprising fatty acid, and a dilute aqueous so-

lution of alkali. For example carrying out this process in a colloid mill of the rotating disc type with variable adjustable clearances using asphalt artificially produced from petroleum, introducing oleic acid (a commercial grade of pale oleine of 100% free fatty acidity) in the form of potash soap, and employing water of hardness between 20 and 25 parts per 100,000 I have investigated the effect of variations in the proportion of the emulsifier on the size of the dispersed bitumen particles in the emulsion.

As a result of these investigations I have found that for variations between 2% and  $\frac{1}{2}\%$  in the proportion of oleine there is practically no change in the average size of the particles in the emulsion. When the proportion of oleine is carried below 0.45% there is a substantial increase in the size of the particles and this continues until the proportion of emulsifier is reduced below 0.36% when no emulsification takes place. For proportions of emulsifier above 0.5% the average size of the bitumen particles has been found to be  $3\mu$  and the proportion of particles above  $8\mu$  in diameter was exceedingly small, while with a proportion of 0.4% emulsifier the average diameter of particles was greatly increased and the proportion of particles above  $8\mu$  in diameter was considerably increased. When the proportion of emulsifier is reduced to an extent (i. e. 0.45% in the particular case referred to above) such that a marked increase in the size of the bitumen particles takes place, the emulsions produced are not sufficiently stable in bulk for industrial use. I have discovered however that such emulsions may be rendered satisfactory by incorporating in them, immediately after their preparation, a stabilizing reagent.

This invention accordingly provides a process for the manufacture of an aqueous emulsion of bitumen having the required balance of stability, which consists in first preparing an unstable emulsion in which the size of the greater proportion of the bitumen particles is relatively large, and immediately after the preparation of such emulsion incorporating therewith a stabilizing reagent. When an emulsion produced by this process

is applied say to a mineral aggregate it breaks down rapidly into its separate constituents, and the bitumen particles being comparatively large coalesce readily to give 5 an effective coating.

The first step in the process according to the invention consists in effecting the emulsification of bitumen with so small a proportion of emulsifier that the size of the bitumen 10 particles in the emulsion is considerably greater than obtains in a stable emulsion.

The proportions of emulsifier suitable for this purpose under one set of conditions are indicated herein. Under other conditions 15 the proper proportions can readily be determined from a few preliminary experiments.

Two examples carried out according to the invention will now be described.

#### 20 Example I

250 grams of Venezuelan asphalt at 110° C. and 125 cc. of neutral potassium oleate solution (containing the equivalent of 1 gram of oleine i. e. 0.4% oleine reckoned on the asphalt) at 70° C. were brought together in a colloid mill and emulsified thereby. The emulsion was run direct from the mill into a vessel containing 125 cc. of 0.5% gelatine solution as a stabilizing reagent. The final 30 product was a coarse emulsion, stable in bulk, of normal viscosity (about 0.15 dynes per square cm.), and giving a quick break on application, accompanied by rapid reformation of the relatively large bitumen particles to 35 produce an adhesive and cohesive film of bitumen.

#### Example II

40 In this example another grade of Venezuelan asphalt was employed. 250 grams of asphalt at 110° C. and 125 cc. of neutral potassium oleate solution (containing the equivalent of 0.5 grams of oleine i. e. 0.2% oleine reckoned on the asphalt) at 70° C.

45 were treated in a colloid mill, and the emulsion was run directly into a vessel containing, as before, 125 cc. of 0.5% aqueous gelatine solution. The product was similar to that obtained in Example I.

50 It is to be noted that in Example II emulsification was in the first place effected with a proportion of oleine as low as 0.2% reckoned by weight on the bitumen. It will be understood that for each particular type and 55 grade of bitumen there will be particular limits (which will vary for different types and grades) in the proportion of emulsifier, within which it is suitable to effect the initial emulsification step according to the invention.

The accompanying drawing shows diagrammatically the comparative size of the dispersed bitumen particles in an emulsion prepared by the present process.

60 Figure 1 is a representation (to a magnifi-

cation of approximately 800 diameters) of a standard emulsion made by the process referred to in the opening part of this specification, that is to say carried out in a colloid mill using Venezuelan asphalt, introducing about 70 2% of oleic acid (reckoned by weight on the bitumen) in the form of potash soap, and employing water of the hardness hereinbefore specified. It will be noted that the proportion of particles having a diameter greater than 75 8μ is practically nil.

Figure 2 is a representation, to the same magnification as Figure 1, of an emulsion made according to Example I. It will be seen that the average size of the particles in this 80 figure is considerably greater than in Figure 1. On a statistical analysis of an emulsion prepared according to Example I it was found that about 25% of the bitumen particles were 85 of a diameter greater than 8μ.

It is an important feature of the emulsion produced according to the present invention, that not only does it break down quickly on application but the time interval between the break and the reformation of the bitumen as a 90 coherent layer with its original physical properties is very materially reduced. It is also a feature of the invention that emulsions produced accordingly possess a normal viscosity, and that the relatively coarse particles 95 of bitumen do not lead to excessive sedimentation.

It has been found that gelatine, glue and other protein and allied substances give satisfactory results as stabilizing reagents in the present process, and a feature of the invention resides in the use of such substances for this purpose. Other stabilizing reagents such as starch and certain other carbohydrates have 100 also been found to give satisfactory results.

The invention is not limited to the carrying out of the process in a colloid mill, nor is it limited to the use of any particular emulsifying agent. The invention covers bituminous materials broadly and includes within its 110 scope the products of the processes described herein.

By the expression "unstable in bulk" as qualifying, in the claims, the stability of an emulsion, I mean to distinguish from an emulsion which is made with a sufficiently large quantity of emulsifying agent to permit the emulsion to maintain its dispersed state, i. e., the state in which it will not coalesce or invert spontaneously over a period of time longer than approximately three months when held in storage.

By the use of the term "an inert stabilizing agent" as employed in the claims, I intend to define such stabilizing agent as starch, gelatin, bentonite, or other well known protective colloids which do not readily react chemically with multivalent ions to change their protective function as is the case with soaps and soap-like materials.

## I claim:

1. A process for the manufacture of an aqueous bituminous emulsion which comprises admixing a bitumen with an aqueous 5 solution of such a small quantity of soap-like emulsifying agent as to produce an initial emulsion having relatively large particle size, bulk in stability and quick breaking characteristics, and thereafter adding an inert stabilizing agent in quantities sufficient to prevent 10 coalescence of the emulsified bitumen particles during storage, whereby to impart bulk stability to the initially formed emulsion, but in insufficient quantities to destroy the quick-breaking 15 characteristics of the emulsion when applied to a porous surface.

2. The process for the manufacture of an aqueous bituminous emulsion which comprises admixing bitumen with an aqueous 20 solution of such a small quantity of soap-like emulsifying agent as to produce an initial emulsion, in which the size of a substantial portion of the dispersed particles is upwards of 10 mu, bulk instability and quick-breaking 25 characteristics, and thereafter adding an inert stabilizing agent in quantities sufficient to prevent coalescence of the emulsified bituminous particles during storage, whereby to impart bulk stability to the initially formed 30 emulsion but of quantities insufficient to destroy the quick-breaking characteristics of the emulsion when applied to a porous surface.

3. An emulsion of bitumen with water as the external phase comprising bitumen and 35 soap-like emulsifying agent present in such a small amount as to produce an initial emulsion of relatively large particle size, but possessing bulk instability and quick-breaking characteristics, and an inert stabilizing agent 40 contained in said emulsion in quantities sufficient to prevent coalescence of the emulsified bitumen particles during storage whereby to impart bulk stability to the initially formed emulsion but of insufficient quantity to destroy 45 the quick-breaking characteristics of the final product when applied to a porous surface.

4. An aqueous bituminous emulsion which comprises bitumen of the type artificially prepared from petroleum, water, and a proportion 50 of soap less than 0.5%, reckoned by weight on the bitumen, the small amount of the soap present producing an initial emulsion having a large particle size of upwards 55 to 10 mu, quick-breaking characteristics and bulk instability, and an inert stabilizing agent present in the emulsion of a quantity insufficient to destroy the quick-breaking characteristics of the relatively large sized bituminous 60 particles when applied to a porous surface.

5. An emulsion of bitumen with water as the external phase comprising bitumen and a soap-like emulsifying agent present in such 65 a small amount as to produce an initial emul-

sion of relatively large particle size, but possessing bulk instability and quick-breaking characteristics, and a gelatinous inert stabilizing agent contained in said emulsion in quantities sufficient to prevent coalescence of the emulsified bitumen particles during storage whereby to impart bulk stability to the initially formed emulsion but of insufficient quantity to destroy the quick-breaking characteristics of the final product when applied 70 to a porous surface.

6. An emulsion of bitumen with water as the external phase comprising bitumen and a soap-like emulsifying agent present in such a small amount as to produce an initial emulsion of relatively large particle size, but possessing bulk instability and quick-breaking characteristics, and a carbohydrate stabilizing agent contained in said emulsion in quantities sufficient to prevent coalescence of the emulsified bitumen particles during storage whereby to impart bulk stability to the initially formed emulsion but of insufficient quantity to destroy the quick-breaking characteristics of the final product when applied 75 to a porous surface.

In testimony whereof I affix my signature.  
LEONARD GOWEN GABRIEL.

95

100

105

110

115

120

125

130